

# United States Patent [19]

Lundberg et al.

[11] Patent Number: **4,665,115**

[45] Date of Patent: \* May 12, 1987

[54] **METHOD FOR CONTROLLING VISCOSITY OF ORGANIC LIQUIDS AND COMPOSITIONS**

[75] Inventors: **Robert D. Lundberg**, Bridgewater; **Robert R. Phillips**, Spring Lake Heights; **Dennis G. Peiffer**, E. Brunswick; **Ilan Duvdevani**, Leonia, all of N.J.

[73] Assignee: **Exxon Research and Engineering Company**, Florham Park, N.J.

[\*] Notice: The portion of the term of this patent subsequent to Oct. 30, 2001 has been disclaimed.

[21] Appl. No.: **781,029**

[22] Filed: **Sep. 27, 1985**

## Related U.S. Application Data

[63] Continuation-in-part of Ser. No. 643,188, Aug. 22, 1984, abandoned, which is a continuation-in-part of Ser. No. 547,908, Nov. 2, 1983, abandoned.

[51] Int. Cl.<sup>4</sup> ..... **C08K 5/01; C08L 39/08**

[52] U.S. Cl. ..... **524/251; 524/385; 524/388; 524/390; 524/504; 524/516; 525/203; 252/33.4**

[58] **Field of Search** ..... **524/516, 504, 390, 385, 524/388, 251; 525/203; 252/33.4**

## References Cited

### U.S. PATENT DOCUMENTS

3,475,358 10/1969 Bixler ..... 524/521  
3,546,142 1/1967 Michaels ..... 524/521  
3,867,330 2/1975 Frisque ..... 524/516

4,118,439 10/1978 Marze ..... 525/203  
4,480,063 10/1984 Lundberg ..... 524/399  
4,552,916 11/1985 Lundberg ..... 524/516  
4,579,671 4/1986 Lundberg ..... 524/516  
4,599,377 7/1986 Duvdevani ..... 524/516

Primary Examiner—C. Warren Ivy  
Attorney, Agent, or Firm—Richard E. Nanfeldt

## ABSTRACT

A method for controlling the viscosity of organic liquids, said organic liquid having a solubility parameter of from about 6 to about 10.5, which comprises incorporating in said organic liquid a minor amount of a polymer complex, said complex being comprised of polymer A, containing neutralized sulfonate groups and polymer B, containing basic nitrogen groups, both functional groups being presented at a level of from about 4 to 500 meq. per 100 g. of polymer, wherein polymer B has the formula:



wherein R<sub>1</sub> is H or an alkyl group having about 1 to about 8 carbon atoms, R<sub>2</sub> is an alkyl group having about 1 to about 18 carbon atoms, x is about 50.0 to 99.8 weight percent and y is about 0.2 to about 50.0 weight percent.

**15 Claims, No Drawings**

## METHOD FOR CONTROLLING VISCOSITY OF ORGANIC LIQUIDS AND COMPOSITIONS

### CROSS-REFERENCE TO RELATED APPLICATIONS

This application is a continuation-in-part of U.S. Ser. No. 643,188, filed Aug. 22, 1984, which is a continuation-in-part of U.S. Ser. No. 547,908, filed Nov. 2, 1983, both now abandoned.

### FIELD OF THE INVENTION

The instant invention relates to a process for controlling the viscosity of organic liquids by incorporating in said liquid a minor amount of two interacting polymers and optionally, a cosolvent for the ionic groups of said polymer. The ionic polymer comprises a backbone which is substantially soluble in said organic liquid, and pendant ionic groups which are substantially insoluble in said organic liquid. The other polymer contains basic nitrogen atoms such as amine groups which interact with the ionic counterion and form a complex. A cosolvent is optionally added which will optionally solubilize the pendant ionomeric groups and provide a reasonably homogeneous mixture of solvent, cosolvent and ionomeric polymer. The preferred compositions prepared by the method of the instant invention comprise an organic liquid having a solubility parameter of from 6 to 10.5 in combination with a sulfonated polymer containing from 0.2 up to 10.0 mole % ionic groups which has been neutralized by a basic material selected from the group consisting of Groups IA and IIA, IB and IIB and also lead, tin and antimony of the Periodic Table of the Elements, wherein the sulfonated polymer is complexed with a polymer containing basic nitrogen atoms such as an amine-containing polymer and optionally, a nonvolatile alcohol or amine as the cosolvent.

### BACKGROUND OF THE PRIOR ART

The rapid decrease in viscosity of liquids with increasing temperature on polymer concentration is well-known. Ideally, for many applications (automobile lubricants, etc.) it would be desirable to solve this problem so that viscosity would be insensitive to temperature or polymer level. Alternatively, it might be desirable to provide liquid systems whose viscosities actually increase with temperature or increase as polymer level is decreased. It is true that with selected polymeric additives, it has been possible to reduce substantially the viscosity change with temperature which does occur with most oils and similar systems. These polymer additives, known as viscosity index improvers (or V.I. Improvers) are generally high molecular weight polymers.

The way in which these additives function can be summarized very briefly. In effect, they perform two functions, i.e., thickening, which merely increases fluid viscosity; and Viscosity Index (V.I.) improvement, which corresponds to limited thickening at ambient temperatures and a correspondingly greater thickening at elevated temperatures. This can be accomplished by utilizing a polymeric additive which is poorly solvated by the liquid at ambient temperatures; however, at elevated temperatures the polymer is more highly solvated such that the polymer expands and is a relatively more effective thickener.

While these V.I. Improvers have proven successful commercially, it is important to note that their effect at reducing viscosity changes with temperatures is rather

mild. For a typical base oil containing a suitable V.I. Improver, the kinematic viscosity will still decrease by a factor of from 5 to 10 as the temperature increases from 30° to 100° C. Obviously, if it is desired to hold the viscosity roughly constant with such temperature changes, current technology has not offered an appropriate additive system. Alternatively, if it is desired to hold viscosity reasonably constant as the polymer concentration is decreased, conventional wisdom has not previously offered that option.

U.S. Pat. No. 3,396,136 describes how copolymers of alkenyl aromatic sulfonic acids, when properly neutralized, can be employed as thickeners for nonpolar solvents. Those metal sulfonate systems have been shown to be very effective; however, when employed as two component systems (i.e., ionic polymer plus nonpolar solvent), the variation of viscosity with increased temperature is very conventional and predictable. That is, the solution viscosity decreases markedly as temperature is increased.

U.S. Pat. No. 3,396,136 further teaches "in situ" neutralization of the sulfonic acid polymer which, under some conditions, can result in the availability of a small amount of polar cosolvent—i.e., a solvent for the sulfonate groups about equal in amount to the amount of sulfonate groups which are present. This amount of polar cosolvent is not within the limits of the instant invention, which only optionally requires amounts of the third component (which interacts with the ionomeric groups of the ionomer copolymer) at levels which range from 10 to 600 times the molar equivalence of ionic groups. This level of cosolvent is about one to two orders of magnitude or more higher than employed in the cited art. In addition, the cited patent is restricted to aromatic sulfonate polymers. The instant invention describes other polymers such as sulfonated ethylene propylene terpolymers, sulfonated Butyl, etc., which are a portion of the polymer complex.

U.S. Pat. No. 3,366,430 teaches the gelling of organic liquids by the interaction of polar "associative bonds" which includes hydrogen bonding and "ionic cross-linking". Again, this patent specifies that two components are necessary—the associating polymer (or polymers in some cases) and the nonpolar organic liquid. There is no mention of a third polar cosolvent except to point out that such polar liquids should not be present. Specifically, this patent states (Column 2, line 7) that the hydrocarbon liquids to which this invention is to be applied should not contain a substantial portion of a miscible protolytic liquid such as methanol. It is clear that the language of this patent limits this invention to gels and further, that any amount of polar liquids which are present to an extent where they disrupt those gels are undesirable. The instant invention is distinct from that cited in that amounts of such polar compounds, as will break up gel at ambient conditions, are often desirable and, in fact the preferred state is free of any said gel at ambient temperatures.

U.S. Pat. No. 3,679,382 teaches the thickening of aliphatic hydrocarbons with synthetic organic polymers which contain olefinically unsaturated copolymerizable acids, amides, hydroxyacrylic esters, sulfonic acids, etc. It is emphasized in this patent (Column 3, line 72) that it is critical that in the preparation of such polymers, no surface active agent, catalyst or other additive be employed which introduces a metallic ion into the system. Therefore, it is preferred to employ ammonium

or amine salts. It is clear that this invention (U.S. Pat. No. 3,679,382) specifically precludes the use of metallic counterions—and is directed towards amine or ammonium derivatives. Metallic counterions are very effective in the instant invention. Finally, this cited patent does describe (Column 7, lines 13-19) that the addition of alcohols will reduce the viscosity of the thickened hydrocarbon and after flow characteristics thereof.

U.S. Pat. Nos. 3,931,021 and 4,118,361 describe the use of ionic polymers and required cosolvents in an organic liquid and V.I. Improvers. The instant invention represents an improvement over U.S. Pat. Nos. 3,931,021 and 4,118,361, and therefore provides a new dimension in viscosity control of hydrocarbon-based solvents. Specifically, it has been discovered that these complexes offer a "flatter" viscosity-temperature relationship than do the sulfonate ionomers previously disclosed. Furthermore, the types of ionic polymers previously described as viscosifiers for oils and low polarity diluents usually are effective thickeners at modest levels, but if one attempts to make a concentrate (10% polymer by weight) the resulting solution is too viscous to handle. The solutions described in this invention can have relatively low viscosities at high concentrations of polymer, yet maintain relatively high viscosities at low polymer concentrations. This change in the viscosity-concentration relationship is a fundamental discovery of potentially great practical relevance. We have indeed observed that this invention is capable of polymer solutions which can be further diluted over broad polymer concentration ranges without a concurrent decrease in solution viscosity—and, in fact, viscosity can actually increase under conditions described herein.

#### SUMMARY OF THE INVENTION

It has been discovered that the viscosity of organic liquids may be conveniently controlled by incorporating in said organic liquid a minor amount of a polymer complex which is the reaction product of a sulfonated polymer and a polymer containing low levels of nitrogen atoms. The polymer complex is characterized as having polymer backbones which are substantially soluble in the organic liquid, and pendant sulfonate groups which are substantially insoluble in the organic liquid.

The number of sulfonate groups contained in the sulfonated polymer of the polymer complex is a critical parameter affecting this invention. The number of sulfonate groups present in the polymer can be described in a variety of ways such as weight percent, mole percent, number per polymer chain, etc. For most polymer systems of interest in this invention, it is desirable to employ mole percent. For vinyl homopolymers, such as polystyrene, the sulfonated analog having a sulfonate content of 1.0 mole percent means on the average that one out of every 100 monomer repeat units in the polymer chain is sulfonated. In the case of copolymers, the same definition applied, except for the purposes of this calculation, the polymer can be considered to be prepared from a hypothetical monomer having an average molecular weight, which is the average of the two monomer components. Similarly for terpolymers, the same averaging concepts apply; however, three components are involved. For example, ethylene-propylene-ethylenedene norbornene (ENB) is a preferred polymer backbone for this invention. A representative terpolymer would have a composition (weight percent) or 50% ethylene, 45% propylene and 5% ENB. This composition has an average repeat unit molecular weight of

about 38.9. Thus, sulfonation of this composition, which occurs at the unsaturation of the ENB units to a level of 1.0 mole %, which means that in 38.9 gms (1 mole of average monomer repeat units) of this polymer, there would be present 0.01 mole of sulfonic acid groups. An alternate way of expressing this is to state the sulfonate level in terms of milliequivalents of sulfonic acid groups per 100 gms of polymer or meq. per 100 g. of polymer. This latter procedure provides a rapid and independent measure of sulfonic acid content in a polymer through simple titration.

Both mole percent sulfonate and milliequivalent of sulfonate will be employed to describe the sulfonate polymers employed in this invention.

In general, the sulfonated polymer will comprise from about 4 meq. up to 500 meq. of sulfonate groups per 100 g. of polymer, more preferably about 10 meq. to about 100 meq. of pendant sulfonate groups per 100 g. of polymer. Sulfonated polymers which are subject to the process of the instant invention are illimitable and include both plastic and elastomeric polymers. Specific polymers include sulfonated polystyrene, sulfonated t-butyl styrene, sulfonated polyethylene, sulfonated polypropylene, sulfonated styrene/acrylonitrile copolymers, sulfonated styrene/methylmethacrylate copolymers, sulfonated block copolymers of styrene/ethylene oxide, acrylic acid copolymers with styrene, sulfonated polyisobutylene, sulfonated ethylenepropylene terpolymers, sulfonated polyisoprene, and sulfonated elastomers and their copolymers such as isoprene-styrene sulfonate copolymer or styrene/butadiene/metal styrene sulfonate terpolymers formed by a free radical copolymerization process.

The sulfonated polymers of the instant invention may vary in number average molecular weight as measured by GPC from 1,000 to 10,000,000, preferably 5,000 to 500,000, most preferably from 10,000 to 200,000. These polymers may be prepared by methods known in the art; for example, see U.S. Pat. No. 3,642,728, hereby incorporated by reference.

Neutralization of the cited sulfonated polymers with appropriate metal hydroxides, metal acetates, metal oxides, etc. can be conducted by means well-known in the art. For example, the sulfonation process as with Butyl rubber containing a small 0.3 to 1.0 mole% unsaturation, can be conducted in a suitable solvent such as toluene with acetyl sulfate as the sulfonating agent. The resulting sulfonic acid derivative can then be neutralized with a number of different neutralization agents such as sodium phenolate and similar metal salts. The amounts of such neutralization agents employed will normally be stoichiometrically equal to the amount of free acid in the polymer plus any unreacted reagent which still is present. It is preferred that the amount of neutralizing agent be equal to the molar amount of sulfonating agent originally employed plus 10% more to ensure full neutralization. The use of more of such neutralization agent is not critical. Sufficient neutralization agent is necessary to effect at least 50% neutralization of the sulfonic acid groups present in the polymer, preferably at least 90%, and most preferably essentially complete neutralization of such acid groups should be effected. The degree of neutralization of said ionomeric groups may vary from 50 to 500 mole %, preferably 90 to 200%. Most preferably, it is preferred that the degree of neutralization be substantially complete, that is, with no substantial free acid present and without substantial excess of the base other than that needed to ensure

neutralization. Thus, it is clear that the polymers which are utilized in the instant invention comprise substantially neutralized pendant groups and, in fact, an excess of the neutralizing material may be utilized without defeating the objects of the instant invention.

We have surprisingly found that a very important factor in determining the strength of the interaction between the amine-containing polymer and the sulfonate-containing polymer is the nature of the counterion. There are, broadly speaking, three major classes of such counterions. The first class, which are less preferred, are those metals of Group I and Group IIA, which include Li, Na, K, etc., Be, Mg, Ca, etc. We have found that these species do not interact as strongly with amine groups as the more preferred species described below. Those metals are commonly defined as members of the transition elements (see chemical text: "Chemical Principles and Properties", by M. J. Sienko and R. A. Plane, McGraw Hill Book Co., 1974, page 19). These metal cations are best exemplified by zinc and interact strongly with pyridine and similar amines. As a consequence, a zinc neutralized sulfonated polymer interacts much more strongly with a styrene/vinyl pyridine copolymer than does a magnesium or sodium neutralized system. It is for this reason that the transition elements are preferred with zinc, copper, iron, nickel and cobalt being especially preferred. We also include antimony and lead as suitable cations.

A third species which is preferred is the free acid of the sulfonated polymer, which will also interact with amine-containing polymers. In this latter case, it is clear that the interaction is a classic acid-base interaction, while with the transition metals, a true coordination complex is created, which is due to the donation of the electron pair of the nitrogen element. This distinction is a very important one and sets these complexes apart from classic acid-base interactions. The surprising observation is that such coordination complexes can form in such extreme dilution insofar as interacting groups are concerned, and that they are apparently formed so far removed from their expected stoichiometry, (based on small molecule analogs).

A variety of polymer backbones will display the desirable properties discovered in this invention:

Sulfonated EPDM

Sulfonate Isoprene Copolymers

Sulfonate SBR Polymers

Sulfonate Butadiene Polymers

Sulfonated Butyl

Sulfonated Acrylate and Methacrylate Copolymers

Sulfonated Block Polymers

Ethylacrylate/Vinyl Pyridine Copolymer and Alkyl

Acrylate Copolymers with Vinyl Pyridine, where the Alkyl group varies in carbon number from 1 to 18

Methyl Methacrylate/Vinyl Pyridine Copolymer and Alkyl Methacrylate copolymers

Sulfonated Polytyrene

Sulfonated Poly-t-butyl Styrene

Sulfonate-containing Copolymers of the above systems with Vinyl Pyridine, wherein the number of carbon groups in the alkyl group varies from 1 to 18 carbon atoms.

Styrene/Vinyl Pyridine Copolymer

Vinyl Pyridine/Styrene/Butadiene Terpolymers

Isoprene/Vinyl Pyridine Copolymer

Butadiene/Vinyl Pyridine Copolymer

Propylene/Vinyl Pyridine Block Copolymer

t-Butyl Styrene/Vinyl Pyridine Copolymers

Vinyl Pyridine Copolymers with alpha-beta ethylenically unsaturated copolymers or terpolymers.

Preferably, the amine content in the basic polymer is

5 expressed in terms of basic nitrogen. In this respect, the nitrogen content in amides and similar nonbasic nitrogen functionality is not part of the interacting species. For example, the amount of vinyl pyridine in the amine-containing polymer can vary widely, but should range 10 from less than 50 weight percent down to at least 0.2 weight percent, more preferably about 0.2 to about 5.0 weight percent in the case of an alkyl methacrylate/vinyl pyridine copolymer or an acrylate/vinyl pyridine copolymer having the formula:



25 wherein  $\text{R}_1$  is H or an alkyl group having about 1 to about 8 carbon atoms,  $\text{R}_2$  is an alkyl group having about 1 to about 18 carbon atoms,  $x$  is about 50 to about 99.8 weight percent, more preferably about 95 to about 99.8 weight percent,  $y$  is about 0.2 to about 50 weight percent, more preferably about 0.2 to about 5.0 weight percent.

30 A minimum of three basic groups must be present on the average per polymer molecule and the basic nitrogen content generally will range from 4 meq. per 100 grams of polymer up to 500 meq. per 100 g. A range of 8 to 200 meq. per 100 g. is preferred.

35 It is evident that the sulfonated polymers covered within this invention encompass a broad class of hydrocarbon polymer systems. It is desirable that these hydrocarbon polymer backbones (in the absence of the sulfonate groups) be soluble in the organic liquid, whose viscosity is to be controlled. To achieve the desired solubility, it is required that the polymer to be employed possess a degree of polarity consistent with that solvent.

40 45 This solubility relationship can be readily established by anyone skilled in the art simply by appropriate texts (e.g., Polymer Handbook, edited by Brandrup and Immergut, Interscience Publishers, 1967, section IV-341). In the absence of appropriate polymer-solvent compatibility knowledge, this can be determined experimentally by observing whether the selected polymer will be soluble in the solvent at a level of 1 gm polymer per 100 ml solvent. If the polymer is soluble, then this demonstrates that it is an appropriate backbone for modification with sulfonate groups to achieve the objectives of this invention. It is also apparent that polymers which are too polar will not be soluble in the relatively nonpolar organic liquids of this invention. Therefore, only

50 those polymer backbones (i.e., as measured in the absence of ionic groups) having a solubility parameter less than 10.5 are suitable in this invention. This precludes the use of such polymers as polyvinyl alcohol, polyacrylonitrile, etc. Also highly crystalline polymers are

55 to be avoided since they tend not to be soluble in the relatively nonpolar organic liquids employed herein. Therefore, acceptable polymers employed in this invention must possess a level of crystallinity of less than

25%. Thus, these acceptable polymers can be considered substantially noncrystalline.

We have also observed that polymers normally insoluble in non-polar solvents such as mineral oils, that the interaction via complexation can induce solubility if one of the polymers is sufficiently soluble.

The preferred ionic EPDM terpolymers for use in the instant invention are prepared by sulfonation of an EPDM-containing ethylenic norbornene units. Other specific examples of preferred ionomeric polymers which are useful in the instant invention include sulfonated polystyrene, sulfonated poly-t-butyl styrene, sulfonated polyethylene, (substantially non-crystalline) and sulfonated polyethylene copolymers, sulfonated polypropylene (substantially noncrystalline), and sulfonated polypropylene copolymers, sulfonated styrene-methyl methacrylate copolymers, (styrene)acrylic acid copolymers, sulfonated polyisobutylene, sulfonated ethylene-propylene terpolymers, sulfonated polyisoprene, sulfonated polyvinyl toluene, sulfonated polyvinyl toluene copolymers and isoprene-styrene sulfonate copolymers formed by a free radical copolymerization process.

The ionomeric polymers of the instant invention may be neutralized prior to incorporation into the organic solvent, or by neutralization of the acid form in situ. For example, preferably the acid derivative is neutralized immediately after preparation. For example, if the sulfonation of polystyrene is conducted in solution, then the neutralization of that acid derivative can be conducted immediately following the sulfonation procedure. The neutralized polymer may then be isolated by means well-known to those skilled in the art; i.e., coagulation, steam stripping, or solvent evaporation, because the neutralized polymer has sufficient thermal stability to be dried for employment at a later time in the process of the instant invention. It is well-known that the unneutralized sulfonic acid derivatives do not possess good thermal stability and the above operations avoid that problem.

The basic nitrogen-containing polymer such as a lauryl methacrylate/vinyl pyridine copolymer of the polymer complex is formed by free radical copolymerization using techniques well-known in the polymer literature. Such polymers can be prepared by a variety of techniques by reacting a basic nitrogen-containing monomer with the alkyl acrylates, or alkyl methacrylates, such as lauryl methacrylate. An emulsion polymerization process is generally preferred, but other processes are also acceptable.

The polymer complex of the sulfonated polymer and the basic nitrogen-containing polymer can be formed by forming a first solution of the sulfonated polymer in an organic liquid and a second solution of the basic nitrogen-containing polymer in the organic liquid, wherein the organic liquid which has a solubility parameter of less than 9.5 and a viscosity of less than about 200 centipoises, as measured at 25° C., and is selected from the group consisting of mineral oil, synthetic oil, alkanes, cycloalkanes, naphthenes and aromatics and mixtures thereof. Alternately both components of the complex can be simultaneously dissolved in the same solvent systems at the desired concentrations. The concentration of the sulfonated polymer in the first solution is about 0.01 to about 10 grams per 100 ml of organic liquid, more preferably about 0.1 to about 5. The concentration of the basic nitrogen-containing polymer in the second solution is about 0.01 to about 10 grams per

100 ml of the organic liquid, more preferably about 0.1 to about 5, and most preferably about 0.1 to about 2. The two solutions of the sulfonated polymer and the basic nitrogen-containing polymer are mixed together to form the polymer complex, wherein either the sulfonated polymer or the basic nitrogen-containing polymer such as lauryl methacrylate vinyl pyridine copolymer can be substantially in excess of the other. The formation of the complex is schematically represented by:



20 The presence of an excess of one component over the other offers a unique opportunity to alter the viscosity-temperature profiles of such solutions. In the creation of the complex a combination of two polymers interacting with an excess of one (such as the lauryl methacrylate/-vinyl pyridine copolymer), we have created a complex which is, in turn, plasticized. Such a system will display modest viscosity at low or ambient temperatures:



35 The application of heat to the right-hand side of Equation 2 would be expected to shift the equilibrium modestly to the left. Consequently, the higher viscosity complex would be favored with a potential increase in solution viscosity.

The weight ratio of the neutralized sulfonated polymer to the copolymer of vinyl pyridinie with an alkyl acrylate or an alkyl methacrylate is 20/1 to 1/20.

40 The polymer complex can be formed *in situ* by the mixing of the solution of the zinc sulfo-EPDM and organic liquid and the solution of the copolymer of vinyl pyridine in the organic liquid or, alternatively, a 45 polymer complex of the zinc sulfo-EPDM and the vinyl pyridine can be dissolved in the organic liquid.

Thus, this concept describes the interaction of two polymers which can give rise to new solution phenomena. A second consequence of this concept is that if such solutions are diluted with non-interactive (less interactive) solvent, such as mineral oil or similar low polarity diluents, the result will be a diminution of the plasticizer component with a relative increase in complex viscosity. Thus, unlike normal polymer solutions which drop off dramatically upon dilution, these solutions may decrease much less in their solution viscosity. Such hydrocarbon or oil solutions have not been available previously. The concentration of the polymer complex in the organic liquid is about 0.01 to about 20 grams per 100 ml, more preferably about 0.1 to about 10, and most preferably about 0.2 to about 10.

The method of the instant invention includes optionally incorporating a cosolvent, for example, a polar cosolvent, into the mixture of organic liquid and polymer complex, to solubilize the pendant sulfonate groups. The polar cosolvent will have a solubility parameter of at least 10.0, more preferably at least 11.0, and may comprise from 0.1 to 40, preferably 0.5 to 20,

weight percent of the total mixture of organic liquid, ionomeric polymer, and polar cosolvent.

While this definition of polar cosolvent is adequate, we also observe that cosolvents with especially long alkyl groups with hydroxyl groups on one or both ends are especially preferred. These cosolvents are based on C<sub>10</sub>-C<sub>30</sub> alkyl chains.

In addition to the requirements for ionic polymer, organic liquid and polar cosolvent, there is the additional and important constraint that the polar cosolvent be more polar than the organic liquid. This is required in order that the proper interaction between polar cosolvent and ionic groups be obtained. If we designate the solubility parameter of the organic liquid as S<sub>L</sub>, and the solubility parameter of the polar cosolvent as S<sub>P</sub>, then we require that:

$$S_P \geq S_L + 1.0$$

In other words, the polar cosolvent will be substantially more polar than the organic liquid to be thickened.

Normally, the polar cosolvent will be a liquid at room temperature, however, this is not a requirement. It is required that the polar cosolvent be soluble or miscible with the organic liquid at the levels employed in this invention. Under normal circumstances, this miscibility requirement precludes the use of water as a polar cosolvent. The polar cosolvent must be present in amounts of from 20 to 600 moles per mole of ionic group in order to give the desirable results of the instant invention and preferably from 30 to 400 moles per mole of ionic group. This level of cosolvent is desirable in creating solutions which can be isoviscous with temperature on concentration.

#### DESCRIPTION OF THE PREFERRED EMBODIMENTS

The following are preferred embodiments of the instant invention.

#### EXAMPLE 1

##### Preparation of Styrene-4-Vinyl Pyridine Copolymer

A copolymer of styrene-4-vinyl pyridine was prepared via a free radical emulsion copolymerization process. The preparation was conducted as follows:

In a suitable, stirred reaction vessel under a nitrogen blanket the following ingredients were charged:

120 ml. distilled water  
50 g. styrene  
3.2 g. sodium lauryl sulfate  
0.1 g. dodecylthiob  
0.2 g. potassium persulfate  
4.7 g. 4-vinyl pyridine

The polymerization was conducted at 50° C. for 24 hours and the resultant emulsion was fluid and uniform. Three ml. of methanol containing 0.1% of hydroquinone was added as an inhibitor and the reaction mixture was precipitated in a large excess of acetone. The precipitate was filtered, then suspended in methanol and blended in a Waring blender to finally disperse the coagulated polymer. The suspension was filtered and dried in a vacuum oven at 60° C. for 24 hours.

The resulting product represented 80% conversion of the reactive monomers and contained 1.68% nitrogen corresponding to 12.5 mole % 4-vinyl pyridine incorporation.

#### EXAMPLE 2

##### Preparation of Sulfonated EPDM

The preparation of sulfonated EPDM has been well-described in the patent and published literature (for example, see U.S. Pat. No. 4,184,988 or ACS Monograph edited by A. Eisenberg, 1980, p. 4). A zinc sulfonated EPDM was prepared via those procedures containing 10 meq. of zinc sulfonate, designated TP 398. The resulting polymer was available as a free-flowing crumb and employed in that form as a blending component in the following examples.

#### EXAMPLE 3

##### Preparation of Polymer Complex

The polymer complex of sulfonated EPDM and polystyrene-Co-4-vinyl pyridine is prepared by charging the required amounts of each polymer to a flask, adding xylene in sufficient quantity to produce the desired concentration and stirring at room temperature until a homogeneous solution is obtained. This generally requires from 2 to 24 hours depending on the concentration required.

#### EXAMPLE 4

##### Comparison of Polymer Complex, Sulfonated EPDM and EPDM Solution Viscosity as a Function of Temperature, With and Without the Addition of Polar Solvent

Solutions were prepared as described in Example 3 of the sulfonated EPDM (10 meq. zinc sulfate)-polystyrene-Co-4-vinyl pyridine complex, sulfonated EPDM (10 meq. sulfonate) and EPDM (backbone EPDM used to prepare the sulfonated EPDM). Viscosity measurements were measured at various temperatures using a Brookfield Viscometer over a range of 0° to 120° C., for each solution. To measured volumes of each solution, various levels of hexanol were added and viscosity vs. temperature obtained. The data are summarized in Table I. The viscosity of the sulfonated EPDM solution shows a marked decrease with increasing temperature. The viscosity of the polymer complex solution shows a much flatter (more isoviscous) temperature relationship. The addition of hexanol to the complex provides an even more temperature insensitive profile. It is important to note that in all cases, the complex behaves quite differently from the sulfonated EPDM-based solutions in terms of the viscosity-temperature relationships.

#### EXAMPLE 5

##### Comparison of Polymer Complex and Sulfonated EPDM Solution Viscosity As A Function of Concentration

Solutions were prepared as described in Example 3 of 5% concentration of sulfonated EPDM (10 meq. zinc sulfonate per 100 g.) in xylene; 5% sulfonated EPDM plus 0.6% polystyrene-Co-4-vinyl pyridine in xylene (Complex A); and 5% sulfonated EPDM plus 1.2% polystyrene-Co-4-vinyl pyridine in xylene (Complex B). Viscosity measurements at 25° C. were obtained of each solution and of xylene dilutions, as noted in Table II.

The data of Table II show that at high concentrations, the solutions containing the complex have relatively lower viscosities as compared to solutions of sulfonated EPDM. On the other hand, the solutions

containing the complex maintain higher viscosities at lower concentrations.

These results are very critical for the following reasons. While ionomer solutions, such as sulfonated EPDM in oil or other hydrocarbons, are very effectively viscosified at high polymer levels (i.e.,  $>1$  or 2%) this very characteristic gives rise to solutions at high polymer levels (5 to 10%) which are too viscous to handle. Yet when such polymers are diluted to low polymer levels ( $\leq 1\%$ ) the viscosity decreases very rapidly and actually becomes less than that of a polymer without ionic groups. Technologically, this is a major deficiency since it is desirable to have viscosification at a very low polymer level. It is evident from the data in Table II that the polymer complexes perform that function. As a consequence, the very desirable result is that the solution viscosity of these polymer complexes can be less variant with polymer concentration than almost any other viscosification approach. Furthermore, the ratios of the polymer components can be altered to vary the viscosity-concentration of the polymer solution at will.

As an example, the data in Table II show that the viscosity of sulfonated EPDM solution at the 5% level is  $9.55 \times 10^5$  cp., while at 1.5% that value is 46 cp, a change of about 20,000. In contrast, the complex, at comparable polymer levels, (4% sulfonated EPDM + 0.96% styrene-vinyl pyridine copolymer) exhibits a viscosity of 8000 cp. The same complex, at a total polymer level of only 1.24%, exhibits a viscosity of 35 cp., a change of only a factor of 200. It is clear that

the change of the solution viscosity of the complex is a factor of 100 less than that of the sulfonate ionomer.

The explanation for this novel behavior is that the ionomer viscosity, at high concentrations, is attributable to interpolymer associations, while at low concentrations, intraassociations occur, which are not effective in viscosification. The complex, however, markedly enhances interpolymer associations, even at dilute polymer levels, and viscosity is thereby enhanced.

#### EXAMPLE 6

##### Polymer Complex With Higher Molecular Weight Polystyrene-Co-4-Vinyl Pyridine Comparing Polymer Complex, Sulfonated EPDM and Polystyrene-Co-4-Vinyl Pyridine Viscosity as a Function of Concentration

A higher molecular weight copolymer of styrene and 4-vinyl pyridine was prepared in a similar manner described in Example 1, by deleting the dodecylthiol from the reaction ingredients.

The resulting product contained 1.13% nitrogen corresponding to 8.4 mole % 4 vinyl pyridine incorporation.

Solutions were prepared in xylene, as described in Example 3, of this higher molecular weight polystyrene-Co-4-vinyl pyridine, and a complex containing 3% (by weight) sulfonated EPDM (10 meq. zinc sulfonate) and 0.72% (by weight) of the polystyrene-Co-4-vinyl pyridine. Viscosity measurements at 25° C. were obtained of each solution and of xylene dilutions as noted in Table III.

TABLE I

| Sample 9234- | Type of EPDM Polymer  | Amount of EPDM Polymer (gms/100 ml) | Styrene-Co-4-Vinyl Pyridine Polymer |              |           |       |      |      | Viscosity (CP) at Temperature (°C.) |      |      |  |  |  |
|--------------|-----------------------|-------------------------------------|-------------------------------------|--------------|-----------|-------|------|------|-------------------------------------|------|------|--|--|--|
|              |                       |                                     | (gms/100 ml)                        | (gms/100 ml) | % Hexanol | 0     | 25   | 50   | 75                                  | 100  | 120  |  |  |  |
| A            | EPDM (NO sulfonation) | 1.5                                 | 0.5                                 | —            | —         | 5.20  | 3.48 | 2.56 | 2.00                                | 1.60 | 1.40 |  |  |  |
| B            | EPDM                  | 1.5                                 | 0.5                                 | 2            | —         | 5.00  | 3.30 | 2.32 | 1.84                                | 1.46 | 1.30 |  |  |  |
| C            | 10 meq. Sulfo-EPDM    | 1.5                                 | —                                   | —            | —         | 5,000 | 135  | 20   | 7.80                                | 4.50 | 3.39 |  |  |  |
| D            | 10 meq. Sulfo-EPDM    | 1.5                                 | —                                   | 2            | —         | 6.96  | 4.96 | 4.05 | 3.40                                | 2.85 | 2.37 |  |  |  |
| E            | 10 meq. Sulfo-EPDM    | 1.5                                 | 0.5                                 | —            | —         | 352   | 166  | 95   | 51                                  | 27.3 | 15.3 |  |  |  |
| F            | 10 meq. Sulfo-EPDM    | 1.5                                 | 0.5                                 | 0.5          | —         | 202   | 127  | 76   | 43                                  | 23.8 | 14.2 |  |  |  |
| G            | 10 meq. Sulfo-EPDM    | 1.5                                 | 0.5                                 | 1            | —         | 83.5  | 75.4 | 56   | 36.3                                | 21.5 | 13.6 |  |  |  |
| H            | 10 meq. Sulfo-EPDM    | 1.5                                 | 0.5                                 | 2            | —         | 30.2  | 31.9 | 29.3 | 23.3                                | 16.1 | 10.5 |  |  |  |

TABLE II

| Solution Viscosity of Polymer and Sulfonated EPDM as a function of Concentration in Xylene |               |                                 |                        |                                 |                             |               |               |
|--------------------------------------------------------------------------------------------|---------------|---------------------------------|------------------------|---------------------------------|-----------------------------|---------------|---------------|
| COMPLEX A                                                                                  |               |                                 |                        | COMPLEX B                       |                             |               |               |
| Sulfo-EPDM (10 Meq, TP398)                                                                 |               | Sulfo EPDM + Sty-Vinyl Pyridine |                        | Sulfo EPDM + Sty-Vinyl Pyridine |                             | Copolymer     |               |
| %                                                                                          | Viscosity cp. | % P-Sty-Co-4-Vinyl Pyridine     | Total Polymer g/100 ml | Viscosity cp.                   | % P-Sty-Co-4-Vinyl Pyridine | Total Polymer | Viscosity cp. |
| 5                                                                                          | 955,000       | 0.6                             | 5.6                    | 120,000                         | 1.2                         | 6.62          | 13,000        |
| 4                                                                                          | 700,000       | 0.48                            | 4.48                   | 48,000                          | 0.96                        | 4.96          | 8,000         |
| 3                                                                                          | 247,000       | 0.36                            | 3.36                   | 39,000                          | 0.72                        | 3.72          | 5,000         |
| 2                                                                                          | 5,000         | 0.24                            | 2.24                   | 10,000                          | 0.48                        | 2.48          | 1,400         |
| 1.5                                                                                        | 46            | 0.18                            | 1.68                   | 2,100                           | 0.36                        | 1.86          | 490           |
| 1                                                                                          | 5             | 0.12                            | 1.12                   | 25                              | 0.24                        | 1.24          | 35            |

TABLE III

| Solution Viscosity of High Molecular Weight Polystyrene-Co-4-Vinyl Pyridine, Sulfonated EPDM and Polymer Complex as a Function of Concentration |               |                                                 |               |                                                        |                |               |
|-------------------------------------------------------------------------------------------------------------------------------------------------|---------------|-------------------------------------------------|---------------|--------------------------------------------------------|----------------|---------------|
| Sulfo EPDM (10 meq. zinc sulfonate)                                                                                                             |               | High Molecular Weight P-Sty-Co-4-Vinyl Pyridine |               | Sulfo-EPDM High M.W. P-Sty-Co-4-Vinyl Pyridine Complex |                |               |
| %                                                                                                                                               | Viscosity, cp | %                                               | Viscosity, cp | % Sulfo EPDM                                           | % P-Sty-Co-4VP | Viscosity, cp |
| 5                                                                                                                                               | 955,000       | 3                                               | 310           | 3                                                      | 0.72           | 1,650,000     |
| 4                                                                                                                                               | 700,000       | 2                                               | 70            | 2                                                      | 0.48           | 680,000       |
| 3                                                                                                                                               | 247,000       | 1                                               | 10.5          | 1                                                      | 0.24           | 160,000       |
| 2                                                                                                                                               | 5,000         | 0.5                                             | 3.5           | 0.5                                                    | 0.12           | 7,200         |
| 1.5                                                                                                                                             | 46            | 0.25                                            | 1.8           | 0.25                                                   | 0.06           | 15.6          |
| 1.0                                                                                                                                             | 5             |                                                 |               |                                                        |                |               |

These data convincingly demonstrate that a combination of the copolymer of styrene and 4-vinyl pyridine with the zinc sulfo EPDM provides a solution whose viscosity is much enhanced over that of either component polymer even though the complex is much lower in concentration. For example, the sulfo EPDM solution has a viscosity of about 5 cp at 1% polymer, the styrene vinyl pyridine copolymer has a viscosity of 10.5 cp at that same concentration, while the complex exhibits a viscosity of over 7000 cp at a total polymer concentration of 0.62%.

Clearly, the complex, even at very dilute concentrations, is a more effective thickening system for hydrocarbon fluids. There are other unique characteristics of these solutions as well, but more importantly these data demonstrate that the complex provides enhanced intermolecular associations and minimizes the intramolecular associations which are counterproductive in the thickening efficiency of the Sulfo EPDM solutions.

#### EXAMPLE 7

(Preparation of Lauryl Methacrylate and Vinyl Pyridine)

In a 500 ml resin kettle, equipped with a teflon stirrer, nitrogen blanket and thermometer charged:

200 g Lauryl Methacrylate  
200 g Distilled Water, previously boiled  
1 g AIBN  
4 g Na lauryl sulfate  
7 g 4-Vinyl pyridine

The polymerization was conducted at about 80° C. for 5 hours. Product mixture was allowed to cool, then filtered slowly overnight obtaining a tough, tacky residue. The residue was dried with a hair dryer several hours, then 19 hours under vacuum at 200° F. Final product is clear, very tough, very low flow and adhesive. Molecular weight as determined from toluene solution viscosity is about 1,400,000.

#### EXAMPLE 8

Preparation of Lauryl Methacrylate Homopolymer

In a 500 ml resin kettle, equipped with a teflon stirrer, nitrogen blanket and thermometer charged:

200 g Lauryl methacrylate  
200 g Distilled water, previously boiled  
1 g AIBN  
4 g Na lauryl sulfate

The polymerization was conducted at about 80° C. for 5½ hours. Reaction product allowed to cool to a clear, viscous mass, the dissolved in 400 ml toluene, washed four times with water. Toluene solution recovered, evaporated and dried at 180° F. to constant weight. Product was light yellow—very viscous, tacky.

15 Molecular weight as determined from toluene solution viscosity is about 1,350,000.

#### EXAMPLE 9

A solution of 1% Sulfo EPDM (Uniroyal 1025, 10 meq, Zn) in xylene was prepared (5 g in 500 ml xylene).

20 To the various weighed amounts (Table IV) of Lauryl Methacrylate-4-Vinyl Pyridine Copolymer in capped bottles, 50 ml of the 1% Sulfo EPDM solution was added. The solutions were stirred to dissolve the copolymer and allow to complex with the Sulfo EPDM.

25 Brookfield viscosity measurements at 25° C. were obtained on each blend solution. The data are summarized in Table IV.

#### TABLE IV

| Sample # | % Sulfo EPDM | Lauryl Methacrylate - 4-Vinyl Pyridine Copolymer |       | Total Polymer Wt. % | Viscosity, cP |
|----------|--------------|--------------------------------------------------|-------|---------------------|---------------|
|          |              | 2827-                                            | g %   |                     |               |
| 35       | 71A          | 1                                                | —     | 1                   | 6.22          |
|          | 71B          | 1                                                | 0.01  | 0.02                | 9.60          |
|          | 71C          | 1                                                | 0.028 | 0.06                | 67.5          |
|          | 71D          | 1                                                | 0.05  | 0.10                | 908           |
|          | 71E          | 1                                                | 0.07  | 0.14                | 3,645         |
|          | 71F          | 1                                                | 0.09  | 0.18                | 4,700         |
|          | 71G          | 1                                                | 0.11  | 0.22                | 5,650         |
|          | 71H          | 1                                                | 0.13  | 0.26                | 7,660         |
|          | 71I          | 1                                                | 0.186 | 0.38                | 7,950         |
|          | 71J          | 1                                                | 0.25  | 0.5                 | 7,390         |
|          | 71K          | 1                                                | 0.374 | 0.75                | 6,700         |
|          | 71L          | 1                                                | 0.5   | 1                   | 5,200         |
|          | 71N          | —                                                | 0.5   | 1                   | 1.5           |

#### EXAMPLE 10

Blends of Lauryl Methacrylate Homopolymer With Sulfo EPDM (10 meq, Zn) in Solution

50 To the various weighed amounts of Lauryl Methacrylate Homopolymer (Table V) in capped bottles, 50 ml of the 1% Sulfo EPDM solution was added. The solutions were stirred to dissolve the Lauryl Methacrylate Homopolymer and Brookfield viscosity (25° C.) obtained.

#### EXAMPLE 11

60 Blend of Lauryl Methacrylate-4-Vinyl Pyridine Copolymer with Sulfo EPDM (10 meq, Zn) in Methanol/Hexane

A solution was prepared containing 1.25 g Sulfo EPDM (Uniroyal 1025), 10 meq, Zn and 1.25 g lauryl-methacrylate-4-vinyl pyridine copolymer in 50 ml of a solvent mixture of 1% methanol/99% Hexane. A cloudy but homogeneous solution was obtained which, then evaporated to dryness and dried at 50° C. in a

forced air oven for 2½ hours, produced a film that was clear and showed no whitening when stretched. The optical clarity of the polymer blend clearly shows a high level of compatibility for this blend due to the amine-zinc interactions.

## EXAMPLE 12

Attempt to Blend Lauryl Methacrylate Homopolymer with Sulfo EPDM (10 meq. Zn) In Methanol/Xylene

To 50 ml of a solvent mixture of 1% methanol/99% hexane was added 1.25 g sulfo EPDM (uniroyal 1025, 10 meq. Zn) and 1.25 g lauryl methacrylate homopolymer and stirred for 5 days. A murky solution was obtained which phase separated on standing into 3 layers—a thick, hazy top layer, a center layer of whitish solids and a bottom layer of clear liquid. This is in contrast to Example 11 in which a blend of the Sulfo EPDM and Lauryl Methacrylate-4-Vinyl Pyridine Copolymer in the same solvent system gave a homogeneous solution which when evaporated produced a clear film.

These observations clearly demonstrate the incompatibility of the methacrylate polymer-sulfo EPDM blend when amine groups are not present to control compatibility, in comparison to the solution where such interactions do obtain.

TABLE V

| Sample # | % | Lauryl Methacrylate - |               | Total Polymer | Viscosity, cP |
|----------|---|-----------------------|---------------|---------------|---------------|
|          |   | Sulfo EPDM            | Homopolymer g |               |               |
| 2827-71A | 1 | —                     | —             | 1             | 6.22          |
| 94B      | 1 | 0.03                  | 0.06          | 1.06          | 6.06          |
| 94C      | 1 | 0.07                  | 0.14          | 1.14          | 6.60          |
| 94E      | 1 | 0.188                 | 0.38          | 1.38          | 7.52          |
| 94F      | 1 | 0.3                   | 0.6           | 1.6           | 9.36          |
| 94G      | 1 | 0.5                   | 1             | 2             | 17.0          |
| 94H      | — | 0.5                   | 1             | 1             | 1.40          |

Since many modifications and variations of this invention may be made without departing from the spirit or scope of the invention thereof, it is not intended to limit the spirit or scope thereof to the specific examples thereof.

What is claimed is:

1. A method for controlling the viscosity of organic liquids, said organic liquid having a solubility parameter of less than 9.5, a viscosity, as measured at 25°C., of less than 200 centipoises and said organic liquid is selected from the group consisting of naphthenates, alkane, cycloalkane and aromatic hydrocarbons and mixtures thereof which comprise incorporating in said organic liquid a polymer complex at a concentration level of about 0.01 to 20 grams of polymer complex per 100 ml. of said organic liquid, said polymer complex being either formed in situ in said organic liquid or being dissolved in said organic liquid, said complex being comprised of polymer A which contains about 4 meq. to 500 meq. of neutralized sulfonate groups per 100 grams of polymer A and polymer B, containing basic nitrogen groups, said basic nitrogen groups about 4 to 500 meq. per 100 g. of polymer B, wherein polymer B has the formula:



5 10 wherein y must, at minimum, have a value sufficient to represent three vinyl pyridine units, R<sub>1</sub> is H or an alkyl group having about 1 to about 8 carbon atoms, R<sub>2</sub> is an alkyl group having about 1 to about 18 carbon atoms, x is about 50.0 to 99.8 weight percent of polymer B and y is about 0.2 to about 50.0 weight percent of polymer B wherein said sulfonate groups of said polymer A have been neutralized with an element selected from the group consisting of transition elements, antimony and lead, said polymer A having a polymeric backbone substantially soluble in said organic liquid and said polymer A having a molecular weight of about 1,000 to 10,000,000.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445

wherein y must, at a minimum, have a value sufficient to represent three vinyl pyridine units, R<sub>1</sub> is H or an alkyl group having about 1 to about 8 carbon atoms, R<sub>2</sub> is an alkyl group having about 1 to about 18 carbon atoms, x is about 50.0 to .99.8 weight percent of said basic nitrogen-containing polymer and x is about 0.2 to about 50.0 weight percent of said basic nitrogen-containing polymer, wherein said sulfonate groups have been neutralized with basic compounds derived from the group consisting of transition elements, antimony and lead, said polymer having a polymeric backbone substantially soluble in an organic liquid having a solubility parameter of less than 9.5 and said sulfonated polymer having a number average molecular weight of about 1,000 to 15 10,000.

12. The composition of claim 11, wherein said basic nitrogen-containing polymer is a lauryl methacrylate-vinyl pyridine copolymer.

13. The composition of claim 12, wherein the weight ratio of said sulfonated polymer to said basic nitrogen-containing polymer is about 20/1 to 1/20.

14. The composition of claim 11 wherein said sulfonated polymer is a sulfonated EPDM terpolymer.

15. The composition of claim 11, wherein said sulfonated polymer is selected from the group consisting of sulfonated polyethylene, sulfonated polypropylene, sulfonated ethylene-propylene copolymers and sulfonated ethylene-propylene-diene terpolymers, wherein the diene is a nonconjugated diene hydrocarbon having from 5 to 15 carbon atoms and sulfonated polystyrene.

\* \* \* \* \*